

# United States Patent Office

2,716,088

Patented Aug. 23, 1955

1

2,716,088

## LUBRICATING OIL COMPOSITION

Louis A. Mikeska, Westfield, and Charles A. Cohen, Roselle Park, N. J., assignors to Esso Research and Engineering Company, a corporation of Delaware

No Drawing. Original application January 16, 1951, Serial No. 206,313. Divided and this application January 2, 1952, Serial No. 264,678

3 Claims. (Cl. 252—33)

This invention relates to an improved process for preparing oil-soluble sulfonic acids and their derivatives which are especially adapted for use as lubricating oil additives.

This invention provides a method for producing oil-soluble sulfonates from specific petroleum white oil fractions. The method comprises chlorinating the white oil, dehydrochlorinating the chlorinated oil and sulfonating the resulting olefins with a sulfonation agent complex.

The white oil utilized is mainly a naphthenic, aromatic free oil (USP petrolatum liquidum heavy) prepared by the well-known exhaustive sulfuric acid treatment of a heavy petroleum distillate to remove substantially all aromatics. The properties of the specific oil utilized have been found to be quite critical in the process of this invention. Physical inspections should lie within the following limits:

|                             |                  |
|-----------------------------|------------------|
| Molecular weight            | 450—600          |
| Specific gravity 60/60° F   | 0.80—0.90        |
| Saybolt viscosity at 100° F | 225—500          |
| Unsulfonated residue        | 100%             |
| Pour point                  | less than 30° F. |

Petroleum fractions outside the range of this oil do not yield satisfactory results, e. g., they either fail to supply appreciable sulfonated products, supply products which are not oil-soluble, or, if soluble, then of low potency as detergents.

In accordance with the process of this invention the specific oil fraction is subjected to a chlorinating operation by passing gaseous chlorine into the liquid mixture while maintaining the temperature of the mixture substantially low, preferably below 100° C. The passage of chlorine into the hydrocarbon mixture is continued until the gain in weight of the hydrocarbon material indicates that the chlorination reaction has proceeded to the extent desired. A ratio of 0.5 mol (one atomic weight) of chlorine per mol of hydrocarbon has been found to effect a satisfactory chlorination of the hydrocarbon. Chlorination in excess of the indicated level results, on subsequent dehydrochlorination and sulfonation, in the obtaining of insoluble and, hence, undesirable polysulfonates, or excessive formation of dienes which have to be eliminated.

When the increase in weight of the white oil indicates that chlorination has proceeded to the desired level, the entire body of the chlorinated material is subjected to dehydrochlorination. This dehydrochlorination is conducted in liquid phase by conventional means, e. g., thermally, by aqueous alkali, by alcoholic KOH, by alkali in glycols, or catalytically through the use of catalysts, such as barium chloride or amines, such as quinoline and collidine, etc., depending upon manipulative advantages. When the dehydrochlorination is done by thermal means alone, the upper temperature limit is 320° C. The other means of dehydrochlorination utilize an upper temperature level of 300° C. and usually result in less undesirable color formation. The gaseous HCl is thus driven off

2

leaving a liquid, predominantly mono-olefinic, product. If excess dienes are present as indicated by the bromine number or the appearance of disulfonates in the final product, these dienes can be removed by reaction with 5 maleic anhydride prior to sulfonation. The olefinic material so produced is referred to as "white oil olefin" in the appended claims.

The olefinic product is then sulfonated, preferably on an equimolar basis. Since these olefins are not sulfonatable by the use of single sulfonation agents, such as sulfuric acid or sulfur trioxide alone, they must be sulfonated by a sulfonation agent complex, e. g., sulfuric acid and acetic anhydride, SO<sub>3</sub> with ethers such as diethyl ether, or dioxane, brom- or chlorosulfonic acids and ethers or dioxane, SO<sub>3</sub> and pyridine and the like, or mixtures of the preceding. It is to be understood that the term, "sulfonation agent complex" connotes complex materials of the nature indicated. A temperature in the range of —20 to 80° C. is maintained during sulfonation. 15 Inert diluents such as chloroform, petroleum naphtha, sulfur dioxide and acetonitrile may be employed. The oil-soluble sulfonic acids which are predominantly in the organic layer are subsequently neutralized usually with caustic soda or soda ash. The sodium soaps are then 20 extracted with aqueous-alcoholic solutions such as 50% aqueous isopropyl alcohol, 50% aqueous ethyl alcohol, etc. The neutralization can also be accomplished with caustic soda in 50% isopropyl alcohol. Unchanged hydrocarbons are removed by extraction with naphtha. The 25 alcoholic solution of the sodium sulfonates is purified, that is, rendered salt-free by dehydration or extraction with sodium sulfate, sodium carbonate, etc., and the solvent removed leaving a salt and oil-free sulfonate. These sodium salts are then converted in oils by a double 30 composition reaction to the corresponding alkaline earth salts when it is desired to use the latter in lubricating oils. The acids may also be neutralized directly with calcium hydroxide, barium hydroxide, nitrogen bases, etc.

The following examples are given to illustrate this 40 invention and include both the processing of the white oils according to this invention and test results on the products as oil-soluble detergents.

### EXAMPLE I

#### Chlorination of white oils

A white oil was made by exhaustively treating an extracted Coastal distillate with excess fuming sulfuric acid, removing sulfonic acids by neutralization and extraction with dilute alcohol, removing solvent and volatile light ends by steaming, then finishing by percolating the oil through Attapulgus clay. Inspections on the feed to the sulfonation unit and on the finished white oil are shown below.

|                                | Distillate   | Finished White Oil |
|--------------------------------|--------------|--------------------|
| Specific Gravity, 60/60, ° F   | 0.8990       | 0.8822             |
| Flash, ° F                     | 435 (O. C.)  | 435 (P.M.)         |
| Viscosity, S. S. U., at 100° F | 538          | 379.               |
| Viscosity, S. S. U., at 210° F | 58.9         |                    |
| Viscosity Index                | 64           |                    |
| A. S. T. M. Pour, ° F          | —5           | —5.                |
| Color                          | 14 1/2 T. R. | +30 UP Say.        |
| Aniline Point, ° F             | 216.7        |                    |
| Unsulfonated Residue           | 90%          | 100%.              |

65 The above-described oil was chlorinated as follows: A three-necked flask equipped with a stirrer, a return condenser and a thermometer was charged with 1227 grams of the oil, the temperature was raised to 70° C. 70 whereupon chlorine was bubbled through the mixture at a rapid rate. Throughout the reaction the temperature was maintained at 70—80° C. When the reaction mixture had

gained 120 grams, the reaction was discontinued and nitrogen was blown through the mixture in order to remove dissolved chlorine and hydrogen chloride. Subsequent weighing showed that 5 grams of volatile products were removed and that the ultimate gain in weight amounted to 115 grams. Without any further purification the product was submitted for analysis and was shown to contain 8.97% chlorine.

## EXAMPLE II

*Dehydrohalogenation of the chlorinated oil*

The chlorinated oil described above was dehydrohalogenated as follows:

Four hundred grams of the chlorinated oil were placed into a three-way flask fitted with a stirrer, a thermometer and a return condenser. The mixture was then heated, with stirring, to 160° C. at which point a rapid evolution of hydrogen chloride took place. When the reaction subsided, the temperature was raised to 190° C. and again maintained at this level until the evolutioned gas had subsided. Finally, the temperature was raised to 310° C. and maintained at this point for 30 minutes. Qualitative tests had now shown that the reaction product was free of organic chlorine. Passage of nitrogen through the mixture which had been maintained throughout the reaction, was continued for another half-hour to remove last traces of hydrogen chloride. The dehydrohalogenated material consisted of 342 grams of dark viscous oil which was distilled from a Claisen flask under 1 mm. pressure. The product distilled as follows:

| Fraction | Temperature Range, ° C. | Weight of Distillate, gm. |
|----------|-------------------------|---------------------------|
| I        | 150-220                 | 5                         |
| II       | 224-226                 | 228                       |
| III      | 226-290                 | 73                        |
| IV       | (1)                     | 27                        |

<sup>1</sup> Undistilled residue.

## EXAMPLE III

*Sulfonation of the unsaturated oil*

A three-way flask equipped with a stirrer, a return condenser, and a dropping funnel was charged with 228 gms. of the dehydrohalogenated oil (fraction II) and 300 ml. hexane. The dropping funnel was charged with 115 gms. of chlorsulfonic acid dissolved in 180 ml. of dry ethyl ether. The acid-ether complex was then added slowly to the reactor at room temperature. No rise in temperature was noted during the addition of the complex. When this operation was completed, the temperature was raised to 40° C. and maintained at this level for about 2 hours.

Finally, the product was transferred into a separatory funnel and diluted with 450 ml. of hexane and time was allowed for the sludge to settle. The sludge was then withdrawn. It weighed 76 gms. and was discarded.

The supernatant hexane solution was treated with 800 ml. of 50% isopropyl alcohol and was neutralized with sodium carbonate. On standing, two layers were obtained. The upper layer consisted of hexane and unreacted white oil. The lower, alcohol-water layer contained the desired soap. The lower layer was extracted twice more with hexane to remove the last traces of oil.

The water-alcohol layer was now saturated with sodium carbonate at 50° C. Two layers were again obtained. The lower layer, which consisted of a water solution of inorganic salts, was discarded. The upper layer, which consisted of an alcoholic solution of the desired sulfonates, was dried on a drum drier. The dry soap thus obtained consisted of 65 grams of light colored solid which proved to be readily soluble in ethyl ether, and in naphthenic as well as in paraffinic lubricating oils. The sulfonate had a combining weight of 537, which indicates a certain amount of polymeric material.

## EXAMPLE IV

*Calcium salt of white oil-olefin sulfonate*

320 grams of 30 wt. per cent solution of the sodium salt of the sulfonate previously described, in an extracted Coastal distillate having a Saybolt viscosity at 100° F. of 105 seconds, were charged to a 2-liter beaker and heated to 95° C. To the oil was then added 150 grams of a pre-heated 20 wt. per cent solution of calcium chloride in water. The mixture was then brought to the boiling point with stirring and heating continued at the boiling point for 15 minutes. Stirring was then stopped and the beaker contents allowed to settle in a steam bath held at 96-98° C. The lower brine layer which separated out was siphoned off, 15 grams of hydrated lime,  $\text{Ca}(\text{OH})_2$  added, and heating and stirring continued until the temperature reached 140° C. At this temperature, 5 grams of a diatomaceous filter-aid was added, the temperature raised to 150° C., and the mixture filtered thru a precoated funnel with the aid of vacuum. A clear fluid product was obtained having the following inspections:

Sulfated ash=5.88 weight per cent

Calcium=1.98 weight per cent

Sulfur=2.20 weight per cent

Alkaline neut. No.=13.6 mg. KOH/gm.

## EXAMPLE V

*Behavior of product in engine tests*

Lauson Engine Tests were made on a series of lubricating oils. The first, the control, was a lubricating oil containing some additives but no detergent additive. The second test was made with an oil of the same composition to which had been added 3 weight per cent of a calcium sulfonate prepared according to this invention. The results of these tests are tabulated below and it is clear from these data that the product of this invention is a superior detergent additive for lubricating oils.

## Lauson Engine Test

| Detergent Additive                               | Varnish Demerit Rating |
|--------------------------------------------------|------------------------|
| Oil I—None                                       | 4.00                   |
| Oil I+White oil olefin-Ca sulfonate <sup>1</sup> | 3.00                   |

<sup>1</sup> 3 weight percent.

These results clearly indicate how the sulfonates produced by this invention minimize undesirable varnish deposits.

The sulfonic acids and sulfonates formed from the white oils by the method described are indicated to be largely non-aromatic compounds containing naphthenic rings, such as 5 carbon rings. The sulfonation forms true sulfonic acids and not acid sulfates from the dehydrochlorinated naphthenes because the sulfonic acids are stable against hydrolysis. The sulfonic acids and sulfonates are also indicated to contain one double bond linkage to the carbon constituent that is joined to the sulfonic acid or sulfonate group. The uniformity of products obtained through the steps taken is surprising, taking into consideration the complex nature of white oils and variations of its chlorinated derivatives. The sulfonates obtained are soluble in high-boiling petroleum oils and are water immiscible.

The products from the process of this invention are thus true sulfonates, i. e., have a C to S linkage and do not undergo hydrolysis after treatment with HCl for four hours. They are thus valuable textile and lubricating oil additives when added in an amount between about 0.1% up to as much as 10% by weight of the oil. The resulting compositions exhibit improved lubricating properties especially in heavy duty service such as encountered in diesel engines, aircraft engines, and the like. Oils containing the compounds of this invention have a de-

tergent action on the parts of the engine that they lubricate and are capable of being used under increased loads and temperatures without causing seizure of bearings or sticking of piston rings by formation of varnish. Oils compounded with these sulfonates also act as rust preventatives in the engine during period of quiescence.

It is to be understood that the invention is not limited to the specific examples which have been offered merely as illustrations since modifications may be made without departing from the spirit of the invention.

This application is a division of Serial Number 206,313, filed January 16, 1951.

What is claimed is:

1. An improved lubricating composition which comprises a major proportion of a mineral lubricating oil and a minor proportion, sufficient to improve the detergency characteristics of said lubricating oil of a naphthenic non-aromatic calcium sulfonate of a white oil olefin, said white oil olefin having a molecular weight in the range of 450 to 600 and being derived from a naphthenic, non-aromatic white oil by chlorination with not more than about 0.5 mol of chlorine per mol of hydrocarbon at an elevated temperature below 100° C., followed by dehydrochlorination.

2. An improved lubricating composition which com- 25

prises a major proportion of a mineral lubricating oil and 0.1 to 10% by weight based on the weight of lubricating oil of a naphthenic non-aromatic calcium sulfonate of a white oil olefin, said white oil olefin having a molecular weight in the range of 450 to 600 and being derived from a naphthenic, non-aromatic white oil by chlorination with not more than about 0.5 mol of chlorine per mol of hydrocarbon at an elevated temperature below 100° C., followed by dehydrochlorination.

10 3. An improved lubricating composition which comprises a major proportion of a mineral lubricating oil and about 3% by weight based on the weight of lubricating oil of a naphthenic non-aromatic calcium sulfonate of a white oil olefin, said white oil olefin having a molecular weight in the range of 450 to 600 and being derived from a naphthenic, non-aromatic white oil by chlorination with not more than about 0.5 mol of chlorine per mol of hydrocarbon at an elevated temperature below 100° C., followed by dehydrochlorination.

References Cited in the file of this patent

UNITED STATES PATENTS

2,203,696 Olin ----- June 11, 1940  
2,361,476 Higbee ----- Oct. 31, 1944